

## UNITED STATES PATENT OFFICE.

GABRIEL N. HARCY, OF LYME, OHIO.

## IMPROVEMENT IN ADHESIVE COMPOSITIONS FOR FLY-PAPER.

Specification forming part of Letters Patent No. 128,223, dated June 25, 1872; antedated June 6, 1872.

Specification of a composition of matter to be called "Harcy's Adhesive Fly-Catcher," invented by GABRIEL N. HARCY, of Lyme, Huron county, Ohio.

Take two and one-fourth pounds of fine pulverized gum copal and beat it up first with seven pounds of castor-oil till it forms a perfect paste; then set it over a gentle heat, which is to be increased until the base of the composition, (copal,) with the vehicle, (castor-oil,) unites so that it looks almost transparent; then add the adjuvant, six and one-half pounds of Burgond resin, (Burgundy pitch,) and one pound of gum turpentine, stirring it from the commencement till the adjuvant (resin and turpentine) are perfectly melted; then remove the composition from the fire or heat, and, while hot, spread it on such paper or other

surface that will not soak or absorb the composition, *ad libitum*, (thick or thin,) leaving all round, say five-eighths of an inch margin, unpasted. This allows room enough to the composition for some extension or spreading, and it will not run out when the prepared paper shall be folded for shipment. The composition I generally make in an earthen vessel.

What I claim as my invention, and for which I desire a patent, is—

The compound, composed of the several ingredients herein mentioned, in the proportions and combined in the manner herein described.

GABRIEL N. HARCY.

Witnesses:

PHIL. N. SCHUYLER,  
SAMUEL ORWIG.